

Aug. 24, 1943.

E. SCHÜTZ

2,327,745

ROTARY CASTING

Filed Sept. 27, 1941

Fig. 1.



Fig. 2.



Fig. 3.



Fig. 4.



Edwin Schütz  
INVENTOR  
BY *O. Schmitz*  
his ATTORNEY.

## UNITED STATES PATENT OFFICE

2,327,745

## ROTARY CASTING

Edwin Schütz, Baden, Switzerland, assignor to  
 Aktiengesellschaft Oederlin & Co., Baden,  
 Switzerland

Application September 27, 1941, Serial No. 412,585  
 In Switzerland August 20, 1940

2 Claims. (Cl. 22—65)

The present invention relates to the art of rotary or centrifugal casting.

The object of the invention is the provision of a method and a device for the coreless casting of several rings in one casting piece which are coaxially arranged so that their circular center lines are located on a rotary surface, for instance in a plane, on a rotary cone or on a sphere.

The rotatable mould provided for this centrifugal ring casting method comprises an annular cavity therein consisting of a number of continuously communicated coaxial chambers corresponding to the number and form of the rings to be cast, whereby at the places of transition from one ring to the next one constrictions are provided, of a width to assure an easy passage of the molten metal into said chambers and the escape of the air.

The accompanying drawing represents four preferred embodiments of the invention, whereby like numerals refer to like parts.

Fig. 1 is an axial section of a rotary casting device, wherein the coaxial rings are arranged in one and the same plane.

Figs. 2 to 4 show different embodiments on axial sections wherein the rings are conically arranged, having their circular center lines located on the surface of a rotary cone.

According to Fig. 1 a disk 2 is fastened to a horizontally journaled shaft 1 which can be put into rapid rotation. Said disk 2 carries at its circumference screws 3 provided with wing nuts and hinged to pins 4 by which a second disk 5 is detachably bolted to the disk 2. The sides of the two disks 2 and 5 facing each other show each a recess 6 and 7, respectively, containing the mould plates 8 and 9, respectively, which are again provided with corresponding cavities 10 according to the ring piece to be cast the total cross section of which may have a rectangular, trapezoid or any convenient form. With a view of saving metal the casting at the places of transition from one ring to the next one may be reduced in thickness by constrictions 11 which must present, however, only a gradual change in the width of the cavity for assuring an easy passage and constant contact of the molten metal with the walls of the mould.

The embodiment shown in Fig. 1 presents a rotary plane  $b-b$ , wherein the concentric rings are disposed. The casting piece has therefore the form of a plate with a central hole. The centrifugal casting takes place when the described device is in rapid rotation by pouring the molten metal through the pouring gate 12

of the disk 5 into the cavity 10 in such a quantity till the cavity 10 is filled over the edge 13.

In Fig. 2 the cross section of the cavity 10 presents as middle line a generating line  $a-b$  of a rotary cone  $a-b-b$  about the axis  $a-c$  and the middle line  $a-b$  may vary from  $10^{\circ}$  to  $70^{\circ}$  and more. The conical arrangement of the mould cavity includes the advantage that the flow of molten metal before reaching the cavity 10, is deviated from the radial plane 14 including the direction of the centrifugal force upon a conical surface  $a-b$  and enters the cavity in a condensed mass along the outer wall thereof, so that the splashing of the same into small particles is essentially avoided. The centrifugal force upon the flow of the molten metal effects an exact filling of the cavity and produces a regular and dense structure. The cone upon which the rings are located may have its apex on the side opposite that shown in the drawing.

The embodiment shown in Fig. 3 presents a construction which is specially adapted to be rotated about a horizontal axis  $f-g$ . The charging of the molten metal takes place through the pouring gate 12. The molten metal runs along the conical surface 15 wherfrom it is deviated into the mould cavity 10. The coaxial rings are located on a conical surface  $d-e$  having an acute apex angle, so that the diameters of the three rings do not much differ from one another.

The embodiment according to Fig. 4 is suitable for rotation about a horizontal as well as a vertical axis  $f-g$ . The mould cavity 10 is arranged on the conical surface  $d-e$ . The molten metal is charged through the pouring gate 12 and follows the conical surface 16 into the cavity 10 of the concentric rings and is freely admitted thereto on the whole length of the circumference of said cavity having the smallest diameter.

For high peripheral speed the device can be arranged below the ground.

It will be understood that the rings after being cast are to be separated by any mechanical process and be worked out into sectional bars by machining.

What I claim is:

1. A rotatable mould for casting several coreless rings by centrifugal action comprising an annular cavity therein consisting of a number of continuously communicated coaxial chambers for generating a corresponding number of rings in one casting piece, said cavity presenting constrictions at the places of transition from one chamber to the next one, the circular center lines of said chambers being located on the sur-

face of a rotary cone coaxial with the axis of rotation of the mould, and a pouring gate for the molten metal communicating on the whole circular length with the chamber, the center line of which has the smallest diameter.

2. A rotatable mould for casting several coreless rings by centrifugal action comprising an annular cavity therein consisting of a number of continuously communicated coaxial chambers for generating a corresponding number of rings in one casting piece, the circular center lines of said chambers having different diameters from one another, while the cross sectional area of each chamber is inversely proportional to the

diameter of its circular center line, said cavity presenting constrictions at the places of transition from one chamber to the next one, which are dimensioned to allow an easy passage of the molten metal and the escape of the air, a pouring gate for the molten metal coaxially arranged with respect to said cavity, and an intermediate passage between said pouring gate and said cavity for deviating the molten metal from the direction of the centrifugal force and communicating on the whole circular length with the chamber, the center line of which has the smallest diameter.

EDWIN SCHÜTZ.